

# UNITED STATES PATENT OFFICE.

WILLIAM HESLOP, OF JOHNSTOWN, PENNSYLVANIA.

## ARTIFICIAL-STONE COMPOSITION.

1,105,905.

Specification of Letters Patent. Patented Aug. 4, 1914.

Application filed October 5, 1912. Serial No. 724,064.

*To all whom it may concern:*

Be it known that I, WILLIAM HESLOP, a citizen of the United States, and a resident of Johnstown, in the county of Cambria and State of Pennsylvania, have invented a new and Improved Artificial-Stone Composition, of which the following is a full, clear, and exact description.

This invention relates to improvements in compounds that are used as a building, paving or facing material, in any form and size, and consists of a body material, sulfur and pine tar.

The body material to be used in connection with the sulfur and pine tar may be gravel, sand, clay, limestone, rock, or any other similar material, preferably pulverized or reduced to small particles. The body material can be used separately with the sulfur and pine tar or together, and it depends on the purpose for which the material is to be used, that is, paving, building or facing, the materials are used all together when a ceramic effect is desired.

When the body material has been reduced to the proper state, the proper amount of sulfur and pine tar is added, and the mixture so formed is heated to a proper temperature, care being taken that during the

process of heating the compound is entirely 30 mixed, so as to form a homogeneous body. The function of the pine tar in the compound is to interblend the particles constituting the body element and to give elasticity to the so-formed compound, while the 35 addition of sulfur to the compound increases its binding qualities, and also increases its hardness.

The proportions I would preferably use are: 85 per cent. of body material, 6 per 40 cent. of sulfur and 9 per cent. of pine tar, but a slight modification in the percentage of the elements forming the compound may be made so as to give more or less elasticity or hardness to the compound to be formed. 45

Having thus described my invention, I claim as new and desire to secure by Letters Patent:

An artificial stone composition comprising substantially 6% of sulfur, 9% of pine 50 tar and 85% of gravel.

In testimony whereof, I have signed my name to this specification in the presence of two subscribing witnesses.

WILLIAM HESLOP.

Witnesses:

ED. E. HOHMANN,  
J. C. SLICK.

Copies of this patent may be obtained for five cents each, by addressing the "Commissioner of Patents.  
Washington, D. C."